

Aug. 17, 1954

D. N. HARNEY  
BINDING TAPE FOR THE EDGES OF MESH  
FLY SWATTERS AND THE LIKE  
Filed June 25, 1951

2,686,746

FIG. 1.



FIG. 2.



FIG. 3.



FIG. 5.



FIG. 4.



Inventor:  
Donald N. Harney  
by his Attorneys  
Howson & Howson

Patented Aug. 17, 1954

2,686,746

# UNITED STATES PATENT OFFICE

2,686,746

## BINDING TAPE FOR THE EDGES OF MESH FLY SWATTERS AND THE LIKE

Donald N. Harney, Moorestown, N. J., assignor  
to E. W. Twitchell, Inc., Philadelphia, Pa., a  
corporation of Pennsylvania

Application June 25, 1951, Serial No. 233,415

3 Claims. (Cl. 154—53.6)

1

A principal object of the present invention is to provide a binding tape possessing the combined attributes of flexibility, desirable bulk, economy of materials and production, and a high degree of durability and resistance to abrasion.

A more specific object of the invention is to provide a binding tape composed essentially of paper which shall have the degree of flexibility and felt-like properties required for effective binding of the edges of wire or other mesh fly swatters.

While the binding tape has an application of primary importance to the production of fly swatters, it will be apparent that it will find other applications where a binding tape of the aforesaid characteristics is required.

The invention will be more readily understood by reference to the attached drawings, wherein:

Figure 1 is a view in perspective showing a section of binding tape made in accordance with the invention, the primary elements being separated at one end to more clearly illustrate the construction;

Figure 2 is a section on the line 2—2, Figure 1;

Figure 3 is a face view of the head portion of a fly swatter bound with tape made in accordance with the invention;

Figure 4 is an enlarged sectional view on the line 4—4, Figure 3; and

Figure 5 is a fragmentary view in perspective of an element of the tape illustrating a modification within the scope of the invention.

With reference to Figures 1 and 2, a tape made in accordance with my invention comprises two primary elements designated 1 and 2 respectively. The element 1 consists of a strip of structurally strong paper of the character of kraft which has been provided with a fine textured crepe so that the strip material, while displaying a relatively even surface texture, still possesses a substantial degree of stretch. Preferably the creped strip will be capable of a stretch in the neighborhood of 100 per cent. This has been found highly suitable for uses involving angular bends of the tape on relatively small radii and of a character more fully explained hereinafter. Lesser or greater degrees of crepe, say of the order of 45 to 55 hills to the inch, may be used and will be found satisfactory for certain purposes to which the tape is obviously well suited.

The other element 2 of the tape structure may be composed suitably of multiple-ply cellulose wadding, preferably spot or otherwise embossed in order to effect a better cohesion between the plies and attached to the kraft strip 1 by adhe-

sive. In the present instance the adhesion of the cellulose wadding element 2 to the kraft paper element 1 is effected by means of a longitudinal strip of adhesive 3 applied to the face of the kraft strip 1, illustrated in Figs. 1, 2 and 5. A series of separate spots or localized areas of adhesive similarly applied may be used in lieu of the continuous strip 3.

The cellulose wadding component of the composite tape thus produced possesses a felt-like quality and confers upon the tape a desirable degree of bulk which adapts the tape well to the function of binding the edges of mesh fly swatters as mentioned above. The cellulose wadding is soft and also possesses a degree of flexibility and compressibility which permits it to conform readily to the shapes to which the tape may be bent. In its application to fly swatters, as illustrated in Figure 3, the tape is doubled around the edges of the wire mesh 4, which forms the head of swatter and which is secured to a handle element 5, and is secured to the mesh by suitable stitching 6. The cellulose wadding on the inner side of the binding embraces the raw edges of the mesh 4 and embeds the cut ends of the wire. The wadding thus provides an effective insulation layer between the sharp ends of the wires of the mesh and the kraft envelope 1 which not only precludes penetration of the envelope by the wires but also cushions the impacts to which the kraft envelope is subjected in the normal use of the swatter.

For binding fly swatters I have found suitable a tape wherein the one component consists of kraft paper of approximately 25 lbs. weight on the basis of 500 sheets, 24"x36", before creping; and wherein the other component consists of a five-ply cellulose wadding wherein the individual ply averages in the neighborhood of 12 lbs. plus or minus 10% on the same basis. The first component is creped in the neighborhood of 45 to 55 hills to the inch and the crepe is highly uniform in character which affords the fine texture previously referred to. It will be understood that the foregoing is by way of specific example and that the invention in its broader aspects contemplates for specific purposes material departures from the figures noted.

In the embodiment illustrated in Figures 1 and 2 and described above, the strip 1 was creped in one direction only, i. e. transversely to the length of the strip. It has been found desirable in some instances to provide this strip also with creping in the opposite or longitudinal direction, as indicated in Figure 5 wherein the strip is indicated

by the reference numeral 1. It is preferred that this longitudinal creping be of the same fine textured character as that previously described. The term "fine texture" as applied herein to the creping is to be understood as defining that character of creping wherein the folds or hills are of such high uniformity and are so closely set as to leave the strip with a relatively smooth or even surface texture.

The use of the aforescribed composite tape confers certain highly desirable and improving properties on fly swatters, particularly of the wire mesh type. The properties of the kraft envelope, for example, combined with the cushioning characteristics of a wadding, produces a tough, abrasion resisting binding superior in durability to many of the textile and plastic tapes heretofore employed, and at a fraction of the cost of the prior tapes. The composite tape of this invention is also soft and resilient to a degree substantially precluding the marring of woodwork and finishes by impact of the swatter. As previously set forth, exposure of the wire ends of the swatter is effectively prevented.

I claim:

1. A binding tape for the edges of mesh fly-swatter heads and the like, said tape consisting solely of structurally strong abrasion resistant paper strip material having a fine textured transverse crepe substantially at right angles to the longitudinal edges of the strip material, said crepe consisting of about 45 to 55 hills to the inch, and

10

15

20

30

cellulose wadding in multi-ply strip form, said wadding being attached to a face of said crepe paper strip material at localized areas only to form with said strip material an integrated composite tape of bulk and thickness materially in excess of that of the paper alone, said tape having a high degree of longitudinal extensibility parallel to the plane of the paper and being capable, after being folded flat on itself along a longitudinal line toward the wadding side thereof, of conforming readily without bunching to short radius bends in the plane of the folded tape.

2. A binding tape according to claim 1 wherein the paper strip material is capable of a stretch in the neighborhood of 100 per cent.

3. A binding tape according to claim 1 wherein the paper strip is creped longitudinally as well as transversely.

References Cited in the file of this patent

UNITED STATES PATENTS

| Number    | Name       | Date           |
|-----------|------------|----------------|
| 1,030,004 | Merrifield | June 18, 1912  |
| 1,554,288 | Madle      | Sept. 22, 1925 |
| 1,774,573 | Spafford   | Sept. 2, 1930  |
| 2,071,347 | Kemp       | Feb. 23, 1937  |
| 2,315,818 | Sackner    | Apr. 6, 1943   |
| 2,414,535 | Kaufman    | Jan. 21, 1947  |
| 2,549,069 | Donofrio   | Apr. 17, 1951  |
| 2,570,614 | Wall       | Oct. 9, 1951   |